

Patented Dec. 15, 1942

2,305,215

# UNITED STATES PATENT OFFICE

2,305,215

## CURING SICCATIVE COMPOSITIONS

Walter W. Durant, Old Greenwich, Conn., assignor to American Cyanamid Company, New York, N. Y., a corporation of Maine

No Drawing. Application October 18, 1939,  
Serial No. 300,017

9 Claims. (Cl. 106—264)

This invention relates to the acceleration of the rate of curing or "seasoning" of siccative compositions such as linoleum and coating compositions.

An object of this invention is to provide accelerators for siccative compositions which will cause such compositions to cure more rapidly. Another object of this invention is to improve the alkali resistance of linoleum floor covering compositions.

These and other objects are attained by incorporating in a siccative composition a substance selected from the group consisting of cyanamide, dicyandiamide, melamine and the methylol derivatives thereof.

The following examples in which the proportions are given as parts by weight are given by way of illustration and not in limitation.

### EXAMPLE 1

#### Parts by weight

|            |     |
|------------|-----|
| Binder     | 30  |
| Wood flour | 30  |
| Whiting    | 20  |
| Lithopone  | 20  |
| Cyanamide  | 0.3 |

These substances with or without a small proportion of drier, e. g. 0.1% cobalt naphthenate, are mixed together, e. g. in an internal mixer. The compacted mass which is delivered from the mixer may be disintegrated, as by a set of "scratch rolls" which comprises rolls having intermeshing teeth projecting from their surfaces. The resulting material is sheeted on calender rolls or optionally it may be further mixed and disintegrated and then calendered. The material may be calendered on to burlap or other fibrous backing if desired. The sheeted material is placed in a stoving oven through which a current of heated air from about 70° C. to about 90° C. is circulated until the material is completely "seasoned," i. e. until the sheet acquires the necessary degree of hardness.

The hardness may be measured by any of the methods generally employed in the manufacture of linoleum. See the Federal Stock Catalogue, section 4, part 5, pages LLL-L-351 et seq., and pages LLL-L-361 et seq., for the method employed herein. The time required for "seasoning" a 2 mm. sheet of the above composition is about six days. The resulting "seasoned" floor covering shows improved alkali resistance. One method of determining alkali resistance is to measure the depth in millimeters to which a 5% solution of sodium hydroxide in water penetrates in one hour at a temperature of 70° F. By this method the alkali resistance of the "seasoned sheets" is about 0.18 mm. penetration.

The "seasoning speed" of a 2 mm. sheet of the same mixture which does not contain cyanamide is about twelve to fourteen days and the alkali

resistance of such a composition is about 0.28 mm. The marked improvement obtained with my composition is outstanding inasmuch as I have found it to be very difficult to improve the alkali resistance by even as little as 0.01 mm.

### EXAMPLE 2

#### Parts by weight

|            |    |
|------------|----|
| Binder     | 35 |
| Wood flour | 30 |
| Whiting    | 20 |
| Lithopone  | 20 |
| Cyanamide  | 3  |

These substances may be mixed and sheeted in the same general manner as the procedure set forth in Example 1. The resulting floor covering sheets "season" or "mature" in about three days and the "seasoned" sheets have an alkali resistance of about 0.11, as compared with a seasoning speed of twelve to fourteen days and an alkali resistance of about 0.28 characteristic of similar compositions which omit the cyanamide.

### EXAMPLE 3

#### Parts by weight

|               |     |
|---------------|-----|
| Binder        | 30  |
| Wood flour    | 30  |
| Whiting       | 20  |
| Lithopone     | 20  |
| Dicyandiamide | 1.5 |

These substances may be mixed and sheeted in the same general manner as the procedure set forth in Example 1. The resulting floor covering sheets "season" in about five days and the "seasoned" sheets have an alkali resistance of about 0.18.

If the proportion of dicyandiamide be increased to about 3 parts by weight in the above formulation, the "seasoning" speed and alkali resistance of such compositions are not substantially different from the values obtained using 1.5 parts of dicyandiamide in said formulation.

### EXAMPLE 4

#### Parts by weight

|                          |    |
|--------------------------|----|
| Binder                   | 30 |
| Wood flour               | 30 |
| Whiting                  | 20 |
| Lithopone                | 20 |
| Dimethylol dicyandiamide | 3  |

This composition may be mixed and sheeted according to the procedure of Example 1. The sheeted composition "seasons" in about six days and has an alkali resistance of about 0.18.

### EXAMPLE 5

#### Parts by weight

|            |     |
|------------|-----|
| Binder     | 35  |
| Wood flour | 30  |
| Whiting    | 20  |
| Lithopone  | 20  |
| Melamine   | 0.3 |

This composition may be mixed and sheeted according to the procedure of Example 1. The sheeted composition "seasons" in about seven to eight days.

## EXAMPLE 6

|            | Parts by weight |
|------------|-----------------|
| Binder     | 30              |
| Wood flour | 30              |
| Whiting    | 20              |
| Lithopone  | 20              |
| Melamine   | 1.5             |

These substances may be mixed and sheeted according to the procedure of Example 1. The resulting floor covering sheets "season" in about five days.

## EXAMPLE 7

|            | Parts by weight |
|------------|-----------------|
| Binder     | 30              |
| Wood flour | 30              |
| Whiting    | 20              |
| Lithopone  | 20              |
| Melamine   | 3               |

If these substances be mixed and sheeted according to the method described in Example 1, the resulting floor covering sheets "season" in about five days and have an alkali resistance of about 0.19.

## EXAMPLE 8

| Pigment:           | Vehicle:                                     |
|--------------------|----------------------------------------------|
| 40% titanium oxide | Linseed oil                                  |
| 30% antimony oxide | 0.04% Co metal (added as cobalt naphthenate) |
| 10% zinc oxide     |                                              |
| 20% asbestos       | 0.6% Pb metal (added as lead naphthenate)    |

The pigment and vehicle are ground together in the volume ratio of 28:72. During this grinding about 3% by weight of cyanamide (based on the vehicle) are added to the mix and ground therewith to form a uniform mixture. The resulting paint composition dries more rapidly than similar compositions which omit the added cyanamide.

## EXAMPLE 9

## White enamel

| Pigment:                              | Vehicle:                             |
|---------------------------------------|--------------------------------------|
| 75% low oil absorption titanium oxide | 50% xylol solution of oxidizing type |
| 20% antimony oxide                    | Phthalic-glyceride-drying            |
| 5% zinc oxide                         | Oil modified resin                   |

The pigment and vehicle are mixed to give a ratio of solid pigment to resin solids equal to 1:1. To this mixture is added about 1-3% of dicyandiamide (based on the weight of the mixture). The mixture is thoroughly ground as by ball milling. The enamel thus produced has a much faster drying speed than that of the same composition in which dicyandiamide is omitted.

## EXAMPLE 10

## Varnish vehicle

|                                        |         |       |
|----------------------------------------|---------|-------|
| Resin "A"                              | pounds  | 100   |
| China-wood oil                         | gallons | 19    |
| Refined raw linseed oil                | do      | 3     |
| "Q" (Gardner-Holdt) bodied linseed oil | gallons | 3     |
| Lead acetate                           | pounds  | 2 1/2 |
| Mineral spirits                        | gallons | 43    |
| Liquid drier (6% cobalt metal content) | gallons | 1/4   |

Resin "A" may be a fatty oil soluble resin such as a phenol-formaldehyde condensate modified with rosin and if desirable partially or completely esterified with glycerol or other alcohol. Otherwise it may be an oil soluble phenol-aldehyde

resin obtainable by reacting formaldehyde with an alkyl or an aryl substituted phenol. The resin, wood oil and raw linseed oil are heated to 480° F. in about twenty minutes. When the resin is dissolved, the temperature is raised to 560° F. in about ten minutes and then gradually to 590° F. and is maintained at this point for three to four minutes or until a heavy drop from a paddle is obtained. This varnish is then checked with the bodied oil and lead acetate, cooled and thinned with mineral spirits. A medium chrome green pigment and about 1-3% of melamine (based on total weight of linseed oil) are ground with this varnish enamel until uniformly dispersed. The ratio of pigment to varnish solids should be 37.5:62.5. Coatings of this varnish enamel dry much more rapidly than similar compositions which do not include the melamine. The melamine apparently overcomes the tendency of the phenolic resin to slow up the drying of the other varnish ingredients. The same effect may be observed if melamine be added to varnishes or the like containing alkyd resins modified with phenol-formaldehyde resins.

The binders used in Examples 1 to 7 may be derived from the drying oils and may be made in any convenient well-known manner, such as the methods described in British Patent 305,856 or the binders may comprise any of the various alkyd resins having siccative properties. For drying oil binders, linseed oil is preferable for economic reasons but other siccative oils may be used such as, for example, menhaden or fish oil, tung oil, China-wood oil, soy bean oil, perilla oil, oiticica oil, Schelber oil, sunflower seed oil, etc. The term "siccative oil" as used herein is intended to include not only the so-called drying oils but also the so-called semi-drying oils. Furthermore it is possible to use mixtures of siccative oils with other fatty oils of the non-drying type.

It may be preferable in the manufacture of linoleum to make use of so-called "scrim-oil" or "shed oil" either alone or fluxed with rosin or other gums or resins and/or mixed with a proportion of the so-called "mechanical oil." Either of these types of oils may be used singly if desired.

In the preparation of the siccative oil binders it is customary to use rosin in admixture with the oil although other substances of the same type may be used, e. g., Kauri gum, Congo gum, ester gum, abietic acid and its esters, pimamic acid, etc.

Other siccative binders which may be used in Examples 1 to 7 are the alkyd resins which have siccative properties. Among these, the drying oil modified reaction products of maleic or fumaric acid with terpenes and polyhydric alcohols are particularly desirable. Other alkyd resins which are modified with drying oils may be used such as the phthalic-glyceride resins, the glycol-maleic resins, and mixed resins such as the phthalic-fumaric-glycol-glyceride resins.

Instead of wood flour and/or the whiting and lithopone used in Examples 1 to 7 inclusive, other fillers or pigments may be used. Examples of such fillers are: cork, cellulose pulp, asbestos, cottonwood tree pulp, walnut shell meal, glass fibers, foliated glass, etc. Among the pigments which may be used are included: lithopone, barites, zinc oxide, titanium oxide, chromates, red lead, white lead, malachite green, chrome green, chrome yellow, Prussian blue, iron oxide, etc. Similarly dyes and lakes may be used if desirable.

It is generally preferable to use driers in the

preparation of the binders. The drier is usually added to the binder during the oxidation process and if desirable additional drier may be added when the binder, fillers, etc., are mixed together. Suitable driers include the oil soluble salts such as the napthenates, resinate and linoleates of cobalt, lead, manganese, zinc, chromium. Only a small proportion of these driers based on the siccative oil content, is generally sufficient, e. g. about 0.005-1%, although larger proportions may be used if desirable. Obviously various mixtures of driers may be used.

The coating compositions shown in Examples 8 to 10 inclusive may be modified by substituting other drying oils or other siccative alkyd resins or modified alkyd resins for those included in the said compositions. Similarly other pigments, fillers, and extenders may be added or substituted for those included in these compositions.

The term "seasoning" as applied to linoleum compositions indicates the process of curing by heating or equivalent treatment to polymerize and/or oxidize the composition to a stage wherein the floor covering is sufficiently hard and resistant to abrasion to be suitable for its intended purpose and yet is still sufficiently flexible to permit the usual bending and rolling required of linoleum. The term "maturing" is similarly used. The term "curing" as applied to coating compositions indicates the process of converting a film thereof to a dry, hard coating.

Other accelerators which may be used include methylol cyanamide and the methylol melamines. The methylol derivatives of these compounds are made by known processes of condensing formaldehyde with the amino compound.

I have found that only a small proportion of these accelerators is generally sufficient, e. g. 0.1-5% of the siccative composition but obviously smaller or larger proportions may be used if desirable.

My accelerators are preferably added during the mixing of the binder with the fillers, etc., although they may be added before or during the oxidation of the binder. If my accelerators are added before or during the oxidation they appear to inhibit somewhat the gelation of the siccative binder. It is to be noted, however, that after gelation my accelerators speed up the curing of the siccative composition.

Obviously many modifications in the processes and compositions described above may be made without departing from the spirit and scope of the invention as defined in the appended claims.

I claim:

1. In a process of curing a composition including a siccative material selected from the group consisting of drying oils and drying oil modified polyhydric alcohol-polybasic acid resins, the step which comprises adding to such a composition about 0.1-5% of a substance selected from the group consisting of cyanamide, dicyandiamide, melamine and the methylol derivatives thereof, said substance acting to accelerate the speed of curing of said composition.

2. In a process for curing a floor covering composition including a siccative material selected from the group consisting of drying oils and dry-

ing oil modified polyhydric alcohol-polybasic acid resins, the step which comprises adding to such a composition about 0.1-5% of a substance selected from the group consisting of cyanamide, dicyandiamide, melamine and the methylol derivatives thereof, said substance acting to accelerate the speed of curing of said composition.

3. In a process of curing a floor covering composition containing a siccative oil binder, the step which comprises adding to such a composition about 0.1-5% of a substance selected from the group consisting of cyanamide, dicyandiamide, melamine and the methylol derivatives thereof, said substance acting to accelerate the speed of curing of said composition.

4. In a process of curing a floor covering composition containing a siccative alkyd resin binder, the step which comprises adding to such a composition about 0.1-5% of a substance selected from the group consisting of cyanamide, dicyandiamide, melamine and the methylol derivatives thereof, said substance acting to accelerate the speed of curing of said composition.

5. In a process of curing a floor covering composition including a siccative material selected from the group consisting of drying oils and drying oil modified polyhydric alcohol-polybasic acid resins, the step which comprises adding to such a composition about 0.1-5% of cyanamide, the cyanamide acting to accelerate the speed of curing of said composition.

6. In a process of curing a floor covering composition including a siccative material selected from the group consisting of drying oils and drying oil modified polyhydric alcohol-polybasic acid resins, the step which comprises adding to such a composition about 0.1-5% of dicyandiamide, the dicyandiamide acting to accelerate the speed of curing of said composition.

7. In a process of curing a floor covering composition including a siccative material selected from the group consisting of drying oils and drying oil modified polyhydric alcohol-polybasic acid resins, the step which comprises adding to such a composition about 0.1-5% of melamine, the melamine acting to accelerate the speed of curing of said composition.

8. In a process of curing a siccative coating composition including a material selected from the group consisting of drying oils and drying oil modified polyhydric alcohol-polybasic acid resins, the step which comprises adding to such a composition about 0.1-5% of a substance selected from a group consisting of cyanamide, dicyandiamide, melamine and the methylol derivatives thereof, said substance acting to accelerate the speed of curing of said composition.

9. A floor covering composition containing a siccative binder including a material selected from the group consisting of drying oils and drying oil modified polyhydric alcohol-polybasic acid resins, and about 0.1-5% of a substance selected from the group consisting of cyanamide, dicyandiamide, melamine and the methylol derivatives thereof, said substance acting to accelerate the speed of curing of said composition.

WALTER W. DURANT.